

Nov. 12, 1968

R. L. CAIN

3,410,084

METHOD OF FORMING CHAIN LINK PLATES

Filed April 25, 1966

2 Sheets-Sheet 1



Inventor:  
Robert L. Cain  
By  
Walter F. Schlegel Jr.  
Charles H. Bassett  
Attest

Nov. 12, 1968

R. L. CAIN

3,410,084

METHOD OF FORMING CHAIN LINK PLATES

Filed April 25, 1966

2 Sheets-Sheet 2



3,410,084

**METHOD OF FORMING CHAIN LINK PLATES**  
Robert L. Cain, West Lafayette, Ind., assignor to Amsted  
Industries Incorporated, Chicago, Ill., a corporation of  
New Jersey

Filed Apr. 25, 1966, Ser. No. 545,121  
5 Claims. (Cl. 59—8)

## ABSTRACT OF THE DISCLOSURE

A method of progressively forming wire stock into chain link plates by forming at a first station, opposed locating grooves to divide the wire into sections, and wherein each section is further formed with narrow medial portions. At a second station the sections are flattened and circular cavities are formed therein. Work at the first and second stations is carried out while in a molten lead bath. The sections are quenched in oil, and at a third station the circular cavities are punched to form pin holes. The sections are separated at a forth station into individual link plates.

This invention relates to a method of forming chain link plates for use in the manufacture of link chain for power transmission and conveying systems.

Heretofore, it has been the practice to punch chain link plates from a metal strip and then to harden the links by special heat treatment and finishing methods. As this method results in a scrap loss of approximately 30 percent, it is an object of the present invention to provide a method for forming chain link plates in which the scrap loss is reduced to approximately one or two percent.

Briefly, the present invention comprises a method in which wire stock is moved step-by-step through several forming dies to form a chain of connected link plates having pin holes therein, the link plates being successively separated from the chain of link plates at the completion of the forming operations. While the wire may be cold formed to provide a chain of connected link plates, it is contemplated that the wire may be formed in a heated condition to improve the physical properties of the link plates.

The invention embodies other novel features which are hereinafter set forth in the specification and claims and illustrated in the accompanying drawings, forming part thereof, wherein:

FIGURE 1 is a schematic plan view illustrating the apparatus for progressively forming wire stock to provide a chain of link plates which are successively severed from the chain at the completion of the forming operations.

FIGURE 2 is a side elevation of the apparatus shown in FIGURE 1.

FIGURE 3 is an enlarged fragmentary view illustrating the first work forming station.

FIGURE 4 is an enlarged view illustrating the second work forming station.

FIGURE 5 is an enlarged section showing the third work forming station.

FIGURE 6 is an enlarged detail view showing the 60 shearing station.

Referring now to the drawings for a better understanding of the invention, the apparatus for transforming chain link plates from S.A.E. 4340 alloy steel round wire stock 2 is shown as comprising a furnace 3 in which the wire stock is heated to a temperature of 1550° F. and then withdrawn from the furnace into a tank 4 containing

2

molten lead maintained at a temperature of up to approximately 1000° F.

The wire stock is moved step-by-step within the lead bath tank 4 to a first forming station 6 and then to a second forming station 7 by means of a conventional stock feed mechanism 8 actuated by a hydraulic power cylinder 9. The first forming station 6 comprises a forming anvil 11 and opposing forming punches 12 and 13 actuated by hydraulic cylinders 14 and 16 to compress a section 17 of the wire therebetween to form a section having end portions 18 and a relatively narrow medial portion 19, as viewed in FIGURE 3. Locating grooves 21 are formed in opposite sides of the wire stock by the forming punches 12 and 13 to receive locator members 22—22 carried by the punches.

The chain of connected link plate sections 17 moves step-by-step from the first station 6 to the second station 7 where they are successively flattened between a mashing punch 23 and the anvil 11 and formed with circular cavities 24, each section being accurately located under the punch 24 by reciprocable locators 26 actuated by hydraulic cylinders 27.

The chain of connected sections 17 moves from the lead bath tank 4 into a quenching tank 28 filled with paraffin oil at a temperature of approximately 120° F. The chain of connected link plate sections 17 then moves through a third station 30 comprising a pin hole punch 29 and a die 31 adapted to punch two pin holes 32 in each section, each section being held in fixed position during the punching operation by means of opposing locators 33 actuated by hydraulic cylinders 34 for engagement in the locating grooves 21.

After the hole punching operation, the chain of connected link plate sections 17 moves step-by-step into a reciprocable shear device 36 where the sections 17 are successively separated from the chain of link sections to complete the formation of finished link plates 37 which then pass through a degreasing device 38.

While a hot working process for forming link plates has been shown and described, it will be understood that the wire 2 may be formed in a cold condition while passing through the several forming stations.

I claim:

1. The method of progressively forming wire stock to fabricate chain link plates, which comprises forming notches at spaced intervals in opposite sides of the wire stock to provide a chain of connected link sections, compressing each link section to provide large end portions connected by a relatively narrow medial portion, mashing each link section to provide flat parallel top and bottom surfaces thereon, punching pin holes in said enlarged end portions, and successively shearing each link section from the chain of link sections, the wire stock being maintained in a molten lead bath at a temperature up to approximately 1000° F. during formation of the chain of link sections.

2. A method according to claim 1 in which the wire stock is quenched in a tank of liquid maintained at a temperature of approximately 120° F.

3. A method according to claim 2 in which the pin holes are punched in the link sections after the quenching operation.

4. A method according to claim 1 wherein the wire stock is moved through the molten bath and thence through liquid paraffin oil at a temperature of the order of 120° F.

5. A method according to claim 4 wherein the pin holes

are punched in the link sections after they have passed  
out of contact with the paraffin oil.

859,387 1/1961 Great Britain.

## References Cited

## UNITED STATES PATENTS

1,670,758 5/1928 Witherow ----- 59-35  
1,881,631 10/1932 Jewett ----- 59-35

5 CHARLES W. LANHAM, Primary Examiner.

G. P. CROSBY, Assistant Examiner.